

1

3,306,699

**PROCESS FOR THE PRODUCTION OF FAST DYEINGS ON CELLULOSE FABRICS**

Bernhard Kramer, Cologne-Braunsfeld, Germany, assignor to Farbenfabriken Bayer Aktiengesellschaft, Leverkusen, Germany, a corporation of Germany

No Drawing. Filed Oct. 9, 1964, Ser. No. 402,927. Claims priority, application Germany, Oct. 10, 1963,

F 40,956

4 Claims. (Cl. 8—26)

The present invention relates to the production of fast dyeings on cellulose fabrics.

It has been found that fast dyeings on cellulose fabrics can be obtained, when a dyeing with the dyestuff of the formula



on native or regenerated cellulose is treated with copper discharging agents. This achieves, inter alia, an improvement in the fastness to water and to washing, and this is unexpected in view of the fact that the cellulose dyeing with this dyestuff (C.I. Direct Black 19=Benzo Fast Black G) is stated to be incapable of being coppered in the Colour Index, 2nd edition, volume 2, page 2332 in conjunction with volume 3, Dyestuff No. 35,255.

The dyestuff can be dyed on cellulose fabrics by itself as well as in the form of a mixture with other toning or accompanying dyestuffs. A number of dyestuffs are frequently employed at the same time in order to produce black colour shades. In mixtures of this type, the proportion of the content of Dyestuff C.I. Direct Black 19 should be at least 20%.



The dyeing is carried out by the usual methods. The same applies to the treatment with copper discharging salts. For this purpose, aqueous solutions of copper sulphate are, for instance, suitable.



The following example is given for the purpose of illustrating the invention.

*Example*

The dyestuff of the formula



65 process which comprises treating with a copper discharging agent a dyeing with the dyestuff of the formula



2

is dyed on a cotton or staple rayon fibre fabric according to the following procedure:

100 g. of cotton yarn or viscose yarn are dyed in a dye liquor of 2 l. which contains 7 to 8 g. of the dyestuff, 40 g. of Glauber's salt or Duisburg sodium sulphate and 2 g. of sodium carbonate (only in the case of dyeing cotton). Dyeing starts at 40° C., the temperature is raised to 80–85° C. within 20 minutes and the bath is left at this temperature for one hour. The yarn is thereafter thoroughly rinsed, first with warm water at 40° C. and then with cold water. It is then coppered in an aqueous bath which contains 3 g. of copper sulphate ( $CuSO_4 \cdot 5H_2O$ ) and 4 g. of 40% acetic acid in 2 l.; the treatment is carried out at 70–80° C. for 20 to 30 minutes. In order to improve the resistance of the coppered dyeing towards washing and abrasion, it is sub-

sequently soaped at 45° C. with 0.5 to 1 g./l. of the sodium salt of a paraffin-sulphonic acid or with 2 to 3 g./l. of Marseille soap, then rinsed in the cold and dried.

25 A cotton dyeing prepared with the use of the dyestuff specified at the start of this example, in the form of its mixture with other toning or accompanying dyestuffs, for instance by use of a mixture of

2 g. of the azo dyestuff 1-amino-4-nitrobenzene-2-carboxylic acid-2-phenylamino-5-hydroxy-naphthalene-7-sulphonic acid, reduced at the nitro groups, treated with phosgene and coppered (concentration 80:100),  
35 3 g. of the dyestuff with the formula specified at the start of this example, and  
3 g. of the dyestuff



can also be coppered with the same result.

I claim:

1. Process for the production of fast dyeings on cellulose fabrics, which comprises treating with a copper discharging agent a dyeing with the dyestuff of the formula



55 on cellulosic fabric.

2. Process according to claim 1, wherein said dyeing is prepared in the presence of a toning dyestuff.

3. Fast dyed cellulose fabrics produced by the proc-



65 process which comprises treating with a copper discharging agent a dyeing with the dyestuff of the formula



4. Cellulose fabric according to claim 3 wherein said dyeing has been prepared in the presence of a toning dyestuff.

**References Cited by the Examiner**

Diserens, The Chemical Technology of 1951, Dyeing and Printing, vol. 2, pages 5, 35 and 36, publ. by Reinhold Publishing Corp., New York.

Knecht et al., The Principles and Practice of Textile Printing, 4th ed., 1952, pages 246, 1034 and 1035, published by Charles Griffin and Co., Limited, London.

Colour Index, 2nd ed. 1956, vol. 2, page 2332, entry C.I. Direct Black 19; Colour Index, 2nd ed., vol. 3, page 3303.

Colour Index, 2nd ed., 1956, vol. 2, pages 2001, 2333, entry C.I. Direct Black 22; vol. 3, page 3306, entry C.I. 35435.

NORMAN G. TORCHIN, *Primary Examiner*.

T. J. HERBERT, JR., *Assistant Examiner*.